

No. 707,170.

Patented Aug. 19, 1902.

J. A. SHINN.

ARTIFICIAL SAND AND METHOD OF PRODUCING SAME.

(Application filed Oct. 21, 1901.)

(No Model.)



WITNESSES

*Roy McDermott*  
*C.W. Downing*

*Joseph A. Shinn*  
INVENTOR  
*by Connally Bros.*  
Attorneys

# UNITED STATES PATENT OFFICE.

JOSEPH A. SHINN, OF PITTSBURG, PENNSYLVANIA.

## ARTIFICIAL SAND AND METHOD OF PRODUCING SAME.

SPECIFICATION forming part of Letters Patent No. 707,170, dated August 19, 1902.

Application filed October 21, 1901. Serial No. 79,462. (No specimens.)

*To all whom it may concern:*

Be it known that I, JOSEPH A. SHINN, a citizen of the United States, residing at Pittsburgh, in the county of Allegheny and State 5 of Pennsylvania, have invented certain new and useful Improvements in Artificial Sand and Method of Producing the Same; and I do hereby declare the following to be a full, clear, and exact description of the invention, such 10 as will enable others skilled in the art to which it appertains to make and use the same.

This invention has relation to the manufacture of an artificial or "slag" sand, and has for its object the production from furnace- 15 slag of an article of manufacture which can be used in the same manner and as a substitute for ordinary sand, either river or pit, in the manufacture of mortar, cement, tiles, brick, &c., and which will not alone possess 20 the usual characteristics of natural sand, but will in addition thereto have advantages not inherent in ordinary sand.

This invention consists in the new article of manufacture and the method of producing the same, as hereinafter described and claimed.

In the accompanying drawing I have shown in a single figure a desirable form of apparatus for carrying my invention into effect. 30 It is well known that the dross or slag from iron-furnaces is a waste product entailing large expense in its removal and necessitating the use of large tracts of land for its storage. Many efforts have been made to 35 utilize this waste product, but, so far as I am aware, with but very little success, principally because the methods employed were so expensive that the product would not realize sufficient to repay the cost.

40 By my method, which is practically cost-less, I produce an article of manufacture far superior to what has heretofore been made and which not alone possesses superior qualities, but the product can be in numerous ways 45 distinguished and readily recognized as different from any slag-sand not made according to my invention. The methods heretofore employed to produce slag-sand have been to take the slag after it has come from the 50 furnace and allowed to cool and crush in

stone-crushers to about the size of ordinary rubble, which is then ground in grinding-rolls, or in some cases the slag while still in a fluid condition is thrown into cold water, the effect of the water being to partially disintegrate the slag, so that it can be passed through the grinding-rolls without the use of the crusher. A serious objection to the use of grinding or rubbing rolls, in addition to their expense, is that the product is not a sharp 55 sand.

I have after a great amount of practical experimenting discovered that I can reduce the slag as it comes from the furnace to a condition of perfect slag-sand by the use of 60 jets of cold water forced against the stream or flow of slag in different directions.

In the drawing I have illustrated a preferred form of apparatus for carrying my invention into effect.

A represents the furnace, and B the opening through which the slag is drawn.

C is the under water-jet, placed as closely as possible to the flowing slag.

D is the upper or outer jet, which is preferably placed slightly above and nearly at right angles to the jet C. These jets C and D are connected with a suitable supply of water under pressure and provided with valves, so that the supply and pressure may 70 be regulated to suit different conditions. A chute or apron E is provided for carrying off the slag after it has been acted upon by the double streams or jets.

As the slag flows from the furnace water 80 is turned onto the jets, preferably at a high pressure—say from fifty to one hundred pounds—and directed onto and through the stream of slag. The effect of the double stream of water on the slag is an instant disintegration and a consequent reduction to a fine sand, the fineness of the sand depending to a considerable extent on the quantity and force of water supplied. This disintegration is not the effect alone of the cooling 85 of the slag by the water, but is aided by the friction of the particles of slag which are driven together by the action of the two streams of water. This I have fully demonstrated by using the water on one side only, 90

70

75

80

90

95

100

and I have found that when a single jet or stream is used a large amount of the slag will not be reduced to sand and must be run through the crusher and rollers before it can 5 be used.

The slag-sand produced by my process can be readily distinguished from other slag-sands in a large number of ways, but most easily by its great density, a bushel of ordinary slag-sand weighing from forty to fifty pounds, while the slag-sand made according to my process will weigh from sixty to seventy pounds.

What I claim as new, and desire to patent, 15 is—

1. The method of reducing slag to a comminuted condition consisting in subjecting the molten slag to two streams of water ap-

plied simultaneously on opposite sides of the slag.

2. The method of producing slag-sand consisting in applying to the stream of slag as it flows from the furnace duplicate jets of water under pressure and on approximately opposite sides of the stream of slag.

3. As a new article of manufacture slag-sand produced solely by the action of water on approximately opposite sides of a stream of molten slag.

In testimony whereof I affix my signature 30 in presence of two witnesses.

JOSEPH A. SHINN.

Witnesses:

MARY M. HEDDEN,  
A. A. CONNOLLY.